

Nov. 27, 1956

F. EISERMANN ET AL

2,772,155

HEAT-RESISTING AUSTENITIC STEEL ALLOYS

Filed Oct. 14, 1953



INVENTORS.

FRIEDRICH EISERMANN.  
WALTER SIEGFRIED.

BY

*K. A. Mayr*

ATTORNEY

1

2,772,155

## HEAT-RESISTING AUSTENITIC STEEL ALLOYS

Friedrich Eisermann and Walter Siegfried, Winterthur, Switzerland, assignors to Sulzer Freres, Societe Anonyme, Winterthur, Switzerland, a corporation of Switzerland

Application October 14, 1953, Serial No. 386,006

Claims priority, application Switzerland October 18, 1952

6 Claims. (Cl. 75—128)

The present invention relates to heat-resisting austenitic steel alloys which, although particularly suitable for castings, in comparison with other steel alloys of about equally high temperature stability are considerably lower in secondary components that are expensive and often difficult to obtain in the desired quantities.

The graph shown in the accompanying drawing illustrates one particular feature of the present invention.

Heat-resisting steel structures can be produced from rolled and forged material or by means of steel castings. Due to the fact that many heat-resisting materials, especially those designed for stresses at high temperature, are difficult to work, the use of steel castings has lately increased.

It has been demonstrated, however, that most of the steel alloys which hitherto have been used in the production of rolled or forged material, are not suitable for the production of castings. More specifically, it has been found that the existing alloys, when cast, lack the favorable mechanical properties they possess when rolled or forged and that castings made therefrom do not satisfy the necessary requirements.

Steel intended for rolling or forging is usually deposited as ingot steel in iron molds, whereas steel for steel castings is poured into refractory molds. At the transition from the liquid into the solid state, ingot steel as well as cast steel passes through a stage of primary crystallization, i. e. a formation of crystals at a well-defined arrangement within the melt, which follows definite rules. In the case of stable austenitic steel these primary crystals remain in existence during the cooling, down to room temperature. In addition, secondary phases occur in the mass at room temperature, which can be distinguished as either phases that separate out above the "solidus" line; that is to say that they cannot be eliminated by means of a solution treatment, or phases that come in existence below the "solidus" line and which, depending upon the temperature, can be completely re-incorporated in the ferrous mass by means of a solution treatment.

The methods employed in further processing ingot steel and cast steel differ insofar, as ingot steel is subjected to a hot or cold plastic deformation step, whereby a crushing and scattering of the secondary phases takes place as well as a unilateral stretching of the primary crystals which produces the well-known lineal structure.

Cast steel, on the other hand, retains the secondary phases and the primary crystals if not subjected to a special heat treatment (solution treatment). The result is a dissimilarity in the mechanical properties of rolled and cast materials because of their different structure, whereby in steel intended for heat-resisting castings a suitable formation of the secondary phases and the size of the austenitic grains is of importance.

2

In contrast to cast steel, because of the subsequent working, even an unfavorable austenitic grain size or secondary phase formation in forged or rolled steel can still result in satisfactory properties of the work piece.

As far as steel castings are concerned, a solution treatment, which leads to the diminution or even the complete disappearance of the secondary phase, cannot be applied because of the danger of deformation of the work pieces while they are cooled down from the necessarily high solution temperatures. On the other hand, rolled and forged material, as a rule, can be subjected, prior to further work, to a solution treatment sufficient to cause disappearance of all phases below the "solidus" line.

The requirements which must be observed in connection with castings from plain steel apply to a still greater extent in the case of steel alloys cast in hot molds, such as, for example, in precision casting. In this instance, particular forms of secondary phases may develop because of differences in the cooling conditions and these secondary phases may be of considerable influence upon the heat resistance of the cast material.

The heat-resisting austenitic steel alloys according to the invention, which are particularly suitable for castings, have the following generic composition:

Carbon ..... 0.05 to 0.45 percent.  
Chromium ..... 16 to 27 percent.  
Nickel ..... 10 to 30 percent.  
30 Cobalt, manganese ..... 6 to 12 percent at approx. equal parts.  
Molybdenum, tungsten, columbium/tantalum ..... 6 to 8 percent, the proportional amounts being 3+ 0.8 percent molybdenum, 2+ 0.8 percent tungsten: 1+ 0.8 percent columbium/tantalum.

Steel alloys of the herein disclosed type may comprise the usual proportions of silicon, phosphorus and sulfur. In order to increase the corrosion resistance, in certain cases a silicon content of up to 2 percent is preferred. These steel alloys may additionally contain 0.1 to 0.2 percent nitrogen. In order to improve their resistance at high heat, boron may be added in an amount of 0.4 percent and up to 1 percent at the most. In the presence of nitrogen, a heat resisting steel according to the invention preferably comprises a total amount of 25 percent of nickel, cobalt and manganese. Moreover, such steel alloys are preferably subjected to an aging process after casting; for example by delaying the cooling of the casting. Furthermore, it is advisable to limit the carbon content of alloys according to the invention to such a proportion that no continuous lattice structure of eutectic phases occurs.

Example 1

A steel of the following specific composition has been found to be particularly suitable:

|                    | Percent |
|--------------------|---------|
| 60 Carbon          | 0.15    |
| Silicon            | 0.8     |
| Manganese          | 4       |
| Chromium           | 18      |
| Nickel             | 17      |
| 65 Cobalt          | 4       |
| Molybdenum         | 3       |
| Tungsten           | 1.5     |
| Columbium/tantalum | 1.5     |
| Nitrogen           | 0.15    |

Castings, produced from steel alloys of the foregoing composition prove to have an endurance of 324 hours until rupture, at a test load of 23 kg./sq. mm. and a test temperature of 700° C.

Notwithstanding that columbium and tantalum, as type related elements, always occur together, in a steel according to the present invention, they may be present singly or jointly.

It is known that heat resistance depends upon the level of the re-crystallization temperature of the ferrous mass, upon the amount and degree of precipitation of the intercalated secondary phases and upon the micro-dispersion phases present in the mass. Taking the foregoing facts in consideration, various steel alloys may be developed according to this invention from the following basic composition:

|          | Percent |
|----------|---------|
| Carbon   | 0.15    |
| Chromium | 18      |
| Nickel   | 25      |
| Nitrogen | 0.2     |

Since any increase in the re-crystallization temperature of the mass and the attainment of the desired precipitation effect are primarily the result of the presence of the elements molybdenum, tungsten and columbium/tantalum, i. e. the type of elements which narrow the dissolving range, the nickel content is adjusted to a proportion of 25 percent in order to obtain a stable austenitic composition. The chromium content depends upon the required corrosion resistance which, if desired, can be further increased by an addition of silicon up to 2 percent. The addition of nitrogen to the basic composition is for the purpose of keeping the nickel ratio down and for attaining the proper precipitation effect.

The preferred way of proportioning the quantitative amounts of the supplementary elements molybdenum, tungsten and columbium/tantalum is to always keep the sum of these elements constant, at not less than 4 percent, but preferably at 6 percent. Moreover, it is to be borne in mind that the carbon content of the alloy must be also balanced with respect to these supplementary elements. As the results of tests conducted with steel alloys compounded according to these limitations, it was found that even small changes in the proportion of the said supplementary elements produce exceedingly great changes in the heat resistance of the alloys.

The following tabulation illustrates the endurance qualities of cast steels comprising the afore-mentioned basic ferrous mass and a total content of 6 percent of the supplementary elements molybdenum, tungsten and columbium/tantalum. The figures given indicate the endurance time at a test temperature of 700° C. and a test load of 23 kg./sq. mm.:

| Steel | Percent ratio of: | Time until<br>rupture<br>(in hours) |
|-------|-------------------|-------------------------------------|
|       | Mo : W : Cb/Ta    |                                     |
| a     | 3.5 : 1.5 : 1     | 72                                  |
| b     | 3 : 2 : 1         | 84                                  |
| c     | 2.5 : 2 : 1.5     | 82                                  |
| d     | 2 : 2 : 2         | 6                                   |
| e     | 3 : 1 : 2         | 10                                  |
| f     | 1.5 : 2 : 2.5     | 8                                   |
| g     | 2.5 : 1 : 2.5     | 10                                  |

The endurance values in the foregoing tabulation show the decisive influence of the relative amounts of these supplementary elements upon the heat resistance of various alloys comprising the same basic mass. Thus, the steel samples a, b, c, containing proportional amounts of molybdenum, tungsten and columbium/tantalum in accordance to the herein claimed invention, have endurance

values which are many times those of the steel samples e, f and g, although the last three samples deviate only to a numerically small degree in the relative amounts of these elements.

After the above-described findings, attempts were made to produce a further increase in the endurance value. Thus, in a first series of tests, part of the nickel content was replaced by cobalt which was added in increasing amounts, up to a maximum of 10 percent. In another test series, part of the nickel of the basic mass was replaced by manganese, likewise in increasing amounts up to 10 percent. These attempts did not produce an appreciable improvement with respect to high-temperature resistance.

However, a surprising improvement in heat endurance is obtained if part of the nickel is substituted by about equal parts of cobalt and manganese, at a proportion of 6 to 12 percent of the combined elements. Thus, the steel described in Example 1 has an endurance value of 324 hours until rupture, at a test temperature of 700° C. and a test load of 23 kg./sq. mm. The accompanying graph illustrates the results of replacing various amounts of the 25 percent of nickel by equal amounts of cobalt and manganese combined and testing the steel under the said conditions (700° C., 23 kg./sq. mm.). The endurance times (in hours) are plotted on the logarithmic scale of the ordinate while the abscissa indicates the Co/Mn content in percent. The sum of the amounts of cobalt and manganese is equal to the amount of replaced nickel and the point of intersection of the two coordinates indicates a nickel content of 25 percent. The plotted curve shows a clearly pronounced maximum in the endurance until rupture if in an alloy of the herein claimed type 8 to 12 percent of the nickel are replaced by 4 to 6 percent of each, cobalt and manganese.

#### Example 2

A further unexpected improvement in the high-temperature resistance of these alloys results from the addition of boron, in an amount from 0.4 to 1.0 percent. Thus, a steel comprising, according to this invention:

|                       | Percent |
|-----------------------|---------|
| Carbon                | 0.15    |
| Silicon               | 0.8     |
| Manganese             | 4       |
| 50 Chromium           | 18      |
| Nickel                | 17      |
| Cobalt                | 4       |
| Molybdenum            | 3       |
| Tungsten              | 2       |
| 55 Columbium/tantalum | 1       |
| Nitrogen              | 0.15    |
| Boron                 | 0.6     |

has an endurance time of 481 hours until rupture at a test temperature of 700° C. and a test load of 23 kg./sq. mm.

It is expedient in many instances to subject steel alloys of this invention to an aging treatment. This can be accomplished by either heat treating the cast in a furnace or as a result of exposure to a normal operation temperature of the device or machine which comprises the cast. Another way of aging consists in extending the cooling period after the casting.

An important property of such alloys is, obviously, the degree of fluidity in casting. It is known that the flow of liquid steel increases with increasing carbon content. On the other hand, higher amounts of carbon may produce a network of eutectic phases with increasing numbers of interconnecting links which may cause a decrease in the high-temperature resistance.

In a steel of this invention good flow properties can be obtained simultaneously with the desired resistance at high temperatures by means of restricting the carbon content to such an extent that no continuous lattice structure of eutectic phases occurs.

The use of a steel according to this invention is not restricted to the production of cast articles. Steel of the herein disclosed composition can be rolled and forged for the subsequent production of heat resisting construction elements.

Having described the invention, what is claimed for the purpose of obtaining Letters Patent is:

1. A heat-resisting austenitic steel alloy particularly suitable for casting articles capable of withstanding severe mechanical stress at high temperatures, said steel alloy containing, a ferrous base, essentially 0.05 to 0.45 percent carbon, 16 to 27 percent chromium, 10 to 30 percent nickel, a total of 6 to 8 percent molybdenum, tungsten and columbium/tantalum, the three last named constituents being present in the following proportions: 2.2 to 3.8 percent molybdenum; 1.2 to 2.8 percent tungsten; 0.2 to 1.8 percent columbium/tantalum, and a total of 6 to 12 percent cobalt and manganese in substantially equal amounts, and incidental impurities.

2. A heat-resisting austenitic steel alloy as defined in claim 1, containing silicon, phosphorus, sulfur, nitrogen, and boron in the conventional proportions.

3. A heat-resisting austenitic steel alloy according to claim 1, containing 0.1 to 0.2 percent nitrogen and the combined amount of nickel, cobalt and manganese being substantially 25 percent.

4. A heat-resisting austenitic steel alloy according to claim 1, containing boron in an amount of 0.4 to 1.0 percent.

5. A heat-resisting austenitic steel alloy, containing in a ferrous base, essentially

|                       | Percent |
|-----------------------|---------|
| Carbon                | 0.15    |
| Silicon               | 0.8     |
| Manganese             | 4       |
| 5 Chromium            | 18      |
| Nickel                | 17      |
| Cobalt                | 4       |
| Molybdenum            | 3       |
| Tungsten              | 1.5     |
| 10 Columbium/tantalum | 1.5     |
| Nitrogen              | 0.15    |

6. A heat-resisting austenitic steel alloy, containing in a ferrous base, essentially

|                    | Percent |
|--------------------|---------|
| Carbon             | 0.15    |
| Silicon            | 0.8     |
| Manganese          | 4       |
| Chromium           | 18      |
| Nickel             | 17      |
| Cobalt             | 4       |
| Molybdenum         | 3       |
| Tungsten           | 2       |
| Columbium/tantalum | 1       |
| Nitrogen           | 0.15    |
| Boron              | 0.6     |

#### References Cited in the file of this patent

#### UNITED STATES PATENTS

|           |               |               |
|-----------|---------------|---------------|
| 2,504,453 | Rotherham     | Apr. 18, 1950 |
| 2,516,125 | Kramer et al. | July 25, 1950 |

#### OTHER REFERENCES

Wartime Report, National Advisory Committee for Aeronautics, Advance Report 4C 22, pages 65 and 71. Edited by Freeman et al. Received at the Patent Office Library Nov. 26, 1948.